

# UNITED STATES PATENT OFFICE.

ALBERT L. CLAPP, OF MARBLEHEAD, MASSACHUSETTS, ASSIGNOR TO THE FLINTKOTE COMPANY, OF BOSTON, MASSACHUSETTS, A CORPORATION OF MASSACHUSETTS.

## PAPER FELT.

1,372,640.

Specification of Letters Patent. Patented Mar. 22, 1921.

No Drawing.

Application filed November 17, 1919. Serial No. 338,765.

*To all whom it may concern:*

Be it known that I, ALBERT L. CLAPP, a citizen of the United States, residing at Marblehead, in the county of Essex and 5 State of Massachusetts, have invented new and useful Improvements in Paper Felt, of which the following is a specification.

This invention has for its object to provide an inexpensive strong pliable "free" 10 and porous paper felt such as can be impregnated with bituminous compounds in the manufacture of roofing or flooring materials. Such felt must be "open" or "free" and highly porous or absorbent, so that it 15 will rapidly absorb such materials as molten asphalt or other relatively heavy and adhesive bituminous compounds. Moreover it must possess considerable strength to withstand the tensile strains to which it is subjected in the saturating and impregnating 20 operations, and it must be pliable, without cracking or breaking when bent.

To produce such paper felt, I employ a mixture of rags, news or waste paper, kraft 25 or sulfite pulp and sawdust.

In practice, I charge a beating engine with hot water, preferably at a temperature of 200° to 212° F., and then add about twenty 30 parts by weight of waste paper such as news print. The beater roll is lifted from the bed plate and is set in rotation until the paper is disintegrated. Then I add about thirty 35 parts by weight of rags and about twenty parts by weight of such chemical wood pulp 40 as sulfite, sulfite screenings, sulfate, or sulfate screenings, preferably sulfate or sulfate screenings. The beater roll is adjusted to the bed plate, and the beating is continued for about twenty minutes. During this operation, about thirty parts by weight of fine 45 sawdust are gradually added to the beater stock. After the stock is thus mixed, it is then ready to be further thinned with water and formed into a web or sheet by any suitable web-forming machine. If desired, the 50 stock may be passed through a Jordan engine prior to its being delivered to the stuff chest or flow box.

Before being added to the beater, the rags 55 and the sulfate pulp are preferably cut or chopped into relatively small pieces, say from one-half inch to one and one-half inches in diameter. The sawdust which is employed is preferably that of hard wood, 60 though soft wood sawdust may be employed,

but in any event it is fine enough to prevent the surface of the felted sheet from having small lumps or projections thereon. In fact, I prefer sawdust capable of passing 60 through about a forty-mesh sieve.

Care should be exercised not to unduly prolong the beating operation, as it tends to reduce the pliability of the stock.

I have found that, by the employment of the materials substantially in the proportions as herein specified, it is possible with one beater to secure a production equal to that of four beaters in which rags alone are used to make the sheet, and further that, the weights of dry stock and the caliper of the 70 finished sheets being equal, the yardage of finished sheet material produced by the stock herein described is much greater than that produced by stock consisting of rag stock alone. I regard the use of sawdust as important inasmuch as it assists in making the sheet free, open and porous, increases the 75 caliper, and in addition provides a smoother surface on the sheet and a greater uniformity in thickness or caliper. The chemical 80 wood pulp, *i. e.*, sulfite, sulfate or screenings, increases the strength of the sheet. The waste paper gives body to the sheet, but, as it tends to harden or stiffen and "close" the sheet, a great proportion thereof 85 should not be employed. Its advantage is cheapness, and, if this is not a consideration, it may be replaced by an equivalent proportion of rags.

The function of the rag fibers is to assist 90 in the felting of the sheet, or the binding of the component fibers thereof together, and to insure the flexibility or pliability of the sheet. A sheet as herein described has decided advantages over one which is produced from rags alone, in addition to those hereinbefore pointed out. That is, in addition to being longer and thicker, it is more 95 porous, and flexible or pliable, and of greater strength. For example, a sheet of 100 paper felt made entirely of rags and having a weight of 42 pounds has a caliper of about 40 and a Mullin-test of about 30. A felted sheet as herein described having a weight of 42, has a caliper of about 48 and a Mullin- 105 test of about 45. Obviously, a sheet comprising in addition to the rags, paper and sawdust alone, has a greater caliper than 40 and a lower Mullin-test than a sheet made of rags alone, say, about 20 to 25. On the 110

other hand, a sheet consisting of rags, paper and chemical wood fiber alone, while having an increased strength, has a decreased caliper and yardage. Thus the function of the 5 chemical wood pulp in the sheet embodying the present invention is to increase the strength of the sheet without decreasing its porosity, flexibility and caliper. A sheet embodying the invention, therefore is better adapted for use in the manufacture of 10 roofing and flooring material. It may be passed more rapidly through the saturating tank, in which the molten asphalt or bituminous compound is contained, and more effectively saturated or impregnated with such compound, as a result of which shingles or shingle strips produced therefrom are less likely to curl or buckle when exposed to the 15 elements.

20 After being thus saturated with a relatively low-melting-point bituminous compound, the sheet is printed for flooring purposes, or, if, desired, is coated with a high-melting-point asphalt or bituminous compound, and may be surfaced with crushed slate or other equivalent mineral. Shingles or shingle strips may be cut from the finished sheet. In lieu of impregnating the dry felt sheet, the asphaltic material, in 25 the form of a nonadhesive emulsion, may be added to the stock prior to its being formed into a web, this step however being herein disclaimed, as *per se* it constitutes no part of my invention.

30 35 While I have herein described what I regard as the best proportions of the several ingredients used in the manufacture of the sheet, I should not regard deviations from those proportions or the substitution of equivalents therefor as constituting a departure from the herein disclosed invention, so long as substantially the same results are secured as herein set forth.

I do not herein claim broadly the employment of sawdust, or of paper, or of both, in 45 admixture with rags, in the production of felt suitable for use in the manufacture of prepared roofing, all as claimed in my application Serial No. 215,891, filed February 7, 1918. 50

What I claim is:

1. An open porous flexible smooth-surfaced sheet of paper felt comprising in addition to rag fiber, finely divided sawdust for increasing the caliper and providing a 55 smooth open porous surface, and a sufficient proportion of chemical wood pulp to offset the decrease in strength caused by the presence of sawdust, all producing a sheet of greater caliper and yardage and not less in 60 strength than one produced by an equivalent weight of rag fiber.

2. An open porous flexible sheet of paper felt, consisting of rag fiber, waste paper, chemical wood pulp and sawdust. 65

3. An open porous flexible sheet of paper felt, consisting of approximately, by weight, thirty parts of rags, twenty parts of waste paper, twenty parts of chemical wood pulp and thirty parts of sawdust. 70

4. The herein described process of making paper felt, which consists in first disintegrating waste paper in water, beating therewith rags and chemical wood pulp, adding sawdust to the mixture, and forming 75 such mixture into a web.

5. The herein described process of making paper felt, which consists in disintegrating waste paper in hot water, then beating rags and chemical wood pulp therewith, 80 during such heating gradually adding fine sawdust to the mixture, and finally forming such mixture into a web or sheet.

In testimony whereof I have affixed my signature.

ALBERT L. CLAPP.